

# United States Patent

Groom

[15] 3,660,889

[45] May 9, 1972

[54] **METHOD OF MAKING A WEAR BLADE FOR AN OIL DRILLING TOOL**

[72] Inventor: William James Groom, Belton, England

[73] Assignee: Lion Oil Tool Holdings (International) Limited, Great Yarmouth, Norfolk, England

[22] Filed: Nov. 3, 1969

[21] Appl. No.: 873,370

[30] **Foreign Application Priority Data**

Nov. 6, 1968 Great Britain ..... 52,689/68

[52] U.S. Cl. .... 29/475, 29/493, 117/127

[51] Int. Cl. .... B23p 17/00

[58] **Field of Search** ..... 29/471.1, 475, 471.3, 488, 29/493, 484, 423; 117/127, 130

[56] **References Cited**

UNITED STATES PATENTS

2,964,420 12/1960 Poorman et al. .... 117/127 X

|           |         |                          |            |
|-----------|---------|--------------------------|------------|
| 3,505,101 | 4/1970  | Koffsky et al. ....      | 117/127 X  |
| 848,161   | 3/1907  | Dierig ....              | 29/484 X   |
| 2,515,191 | 7/1950  | Carpenter et al. ....    | 29/471.1   |
| 3,248,788 | 5/1966  | Goldstein et al. ....    | 29/493     |
| 3,258,955 | 7/1966  | Lindsay. ....            | 29/423 X   |
| 3,453,719 | 7/1969  | Feinstra. ....           | 29/472.9   |
| 3,535,767 | 10/1970 | Doherty, Jr. et al. .... | 29/497.5 X |

*Primary Examiner*—John F. Campbell

*Assistant Examiner*—Richard Bernard Lazarus

*Attorney*—Wenderoth, Lind & Ponack

[57] **ABSTRACT**

A method of making oil drilling tools, particularly stabilizers, and wear blades therefor. The blades are made and dressed on a separate former to avoid pre-heating the tool body. They are then welded to the tool body by a low heat electric welding technique and are arranged around the body equally spaced and skewed in an anti-clockwise direction, the total circumferential coverage being complete. Typically there are four blades each skewed 90°.

**4 Claims, 4 Drawing Figures**



PATENTED MAY 9 1972

3,660,889

FIG. 1.



FIG. 2.



FIG. 3.



FIG. 4.



WILLIAM JAMES GROOM, Inventor

BY, *Wendworth, Lind & Ponack*  
Attorneys

**METHOD OF MAKING A WEAR BLADE FOR AN OIL DRILLING TOOL**

The invention relates to oil drilling tools, namely to tools for use in drilling for oil or natural gas. Particular application for the invention is found in stabilizers, turbine drills and pipe-cutting tools.

Oil drilling tools are subject to severe wear and are generally provided with facings of hard, wear resistant metal applied to the steel body of the tool. Problems are presented by the initial application of such facings and more particularly by the replacement of worn facings. The present invention seeks to alleviate these problems.

According to the invention there is provided a method of making a wear blade for an oil drilling tool consisting in forming on a cylindrical former a blade base which comprises a length of steel of substantially rectangular cross-section extending along the former and skewed around it in an anti-clockwise direction substantially 90° or less; applying a dressing of hard wear material to the outer face of the base; and removing the completed blade from the former.

The hard wear material may comprise hard metal carbides bonded in a matrix of brass, the carbides representing preferably 60 to 90 percent or more of the total.

The invention includes within its scope a wear blade when made by the foregoing method and also a method of dressing an oil drilling tool with a plurality of such wear blades, which method consists in applying the blades to a cylindrical steel body part of the tool of the same dimensions as the former and electrically welding the blades to the body part with the use of a low heat input electrode, a welding technique being used which requires preheating to no more than about 300°C, the blades being evenly spaced apart and the number of blades being chosen in relation to their angle of skew so that the blades cover the complete circumference of the body part.

Preferably the electrode is a low heat input high elongation electrode of hydrogen-controlled austeno-ferritic structure.

The method may be used in the replacement of worn blades and as an important aspect of the invention it is proposed that in applying new facings to an oil drilling tool the worn facings are not removed but new blades in accordance with the invention are welded in place adjacent the old facings. Indeed, it may be expedient to increase the effective gauge size of the tool by applying new, thicker blades in this way even if the old blades are not worn.

Preferably the total circumferential coverage of the blades is 360°; it may be rather more but should be no less. In a preferred embodiment there are four blades each skewed 90°. However, there may be more than four blades — perhaps as many as eight. Such blades would be correspondingly narrower and would be correspondingly skewed less. For example, in a six-bladed arrangement each blade would be skewed some 60°.

The invention will further be described with reference to the accompanying drawings, of which:

FIGS. 1 and 2 are schematic diagrams illustrating respectively the manufacture of a wear blade and the application of the blade to a tool in accordance with the invention;

FIG. 3 is a plan view of an oil drilling tool in accordance with the invention; and

FIG. 4 is a plan view of a wear blade in accordance with the invention.

Referring to FIG. 1 the wear blade is made by forming a mild-steel base 1 on a cylindrical former 2 and dressing one side of the base by brazing to it a facing 3 of hard wear material. "ION ALLOY" overlay rods and "IONUX" flux are used to braze the facing 3 to the base 1. The hard wear material may be that known as "IONITE", which is comprised of fragments of sintered tungsten carbides with additives of titanium, tantalum and other hard metal carbides bonded with cobalt in a brass base, the proportions of carbides to base being in the range 60 to 90 percent or more of the whole. Subject to the

maintenance of adequate stability, the higher the proportion of carbide material in the hard wear material the better. The carbide material has a hardness range of from 950 to 1850 Vickers diamond pyramid hardness. The thickness of the facing 3 is about one-fourth inch. The former 2 is the same size and shape as the tool to which the blade is to be applied. In this case the tool is a stabilizer. After forming, the blade is removed from the former.

Referring now to FIG. 2 the blade of FIG. 1 is shown applied to the body 4 of the stabilizer. The body is of EN 24T or EN 19T heat treated steel and the base 1 is welded thereto by means of a low temperature electric welding technique. Electrodes of the kind known as "IONECT" special low heat, maximum elongation electrodes are used to weld the blade to the body 4, the weld metal being shown at 5 in FIG. 2. The "IONECT" electrode is of hydrogen controlled austeno-ferritic structure. The welding process requires a pre-heating temperature of normally no more than 250°C and certainly no more than 300°C.

FIG. 3 shows a stabilizer fitted with the blades. The tool has a "fishing" neck 6 some 28 inches long, an upset portion 7, 18 inches long and a nose 8, 20 inches long. The cylindrical upset portion is provided with four blades 9, each extending from end to end of portion 7 and skewed around the upset portion through 90° in an anti-clockwise sense. The four blades together thus extend around the whole circumference.

FIG. 4 shows the nature of a blade. Each blade comprises a steel base 10 provided with a tungsten carbide facing 11. From the "fishing" neck end the blade is of even thickness for the first 12 inches to 14 inches, whereafter it tapers downwardly in thickness to the nose end. The blades are welded to the upset portion 7 in the manner described with reference to FIG. 2.

It will be seen that when the blades wear down, or if perhaps the effective outside diameter of the tool is to be increased, new or thicker blades may be welded into position adjacent and between the old blades.

Use of the invention as exemplified in the foregoing description made with reference to the accompanying drawings has many advantages. Firstly, it is found that the tools have a particularly long life. Secondly, the wear blades, being capable of being welded to the drilling tools by low temperature techniques, offer the possibility of application to the tools on site at the drilling rig. This means that spares may be held more readily, freight costs are reduced and so is the out-of-service time for a particular tool. Also, spares with a range of inside and outside diameters may be kept to cover a range of possible applications. Furthermore, the tool is not subjected to the high temperatures normally applied for welding, dressing or re-dressing the hard facing metal. This often requires high temperature pre-heating and post-heating to stress-relieve the welds, resulting in deterioration of the blade and tool body by undesired heat treatment. The lower welding temperatures used in the preferred method above described do not appreciably affect the hardness of the tool body.

I claim:

1. A method of making a wear blade for an oil drilling tool consisting in forming on a cylindrical former a blade base which comprises a length of steel of substantially rectangular cross-section extending along the former and skewed around it in an anti-clockwise direction at most substantially 90°; applying a dressing of hard wear material to the outer face of the base; and removing the completed blade from the former.

2. A method as claimed in claim 1 wherein the hard wear material is composed of hard metal carbides bonded in a matrix of brass, the carbides representing 60 to 90 percent or more of the total.

3. A method as claimed in claim 2 wherein the hard wear material is brazed to the base.

4. A method as claimed in claim 1 wherein the hardness of the hard wear material is between 950 and 1850 Vickers diamond pyramid hardness.

\* \* \* \* \*